

## UNITED STATES PATENT OFFICE

HUGH RODMAN, OF OAKMONT, PENNSYLVANIA, ASSIGNOR TO RODMAN CHEMICAL COMPANY, OF VERONA, PENNSYLVANIA, A CORPORATION OF PENNSYLVANIA

## QUENCHING OILS

No Drawing.

Application filed May 16, 1929. Serial No. 363,716.

This invention relates to quenching oils for use in cooling red hot steel, and the like, and particularly to means for improving the quenching action of mineral oils.

5 A major object of the invention is to increase the initial quenching speed of certain mineral oils, particularly those of low viscosity and low flash point by the addition thereto of a small amount of other material, 10 without materially increasing the total cost.

In Patent No. 1,535,379 there is disclosed a method of increasing the initial quenching speed of low-viscosity low-flash mineral oils by adding thereto a small amount of high-viscosity high-flash mineral oil. The present invention is an improvement upon that described in the patent, and is predicated upon the further discovery that the results described in the patent may be improved upon 20 and more economically obtained by adding to mineral quenching oils of low viscosity and low flash point a small amount of the residuum obtained in the distillation of certain high-viscosity high-flash mineral oils, and particularly the residuum obtained when such oils are distilled in vacuo. The resulting accelerated initial quenching effect of the treated oil is apparently due to some substances in the added residuum that does not 30 pass off in distilling processes.

The term "residuum" is here used to denote the solid or semi-solid tacky substance left in the stills after distilling off all material which can properly be called oil. The term is not to be confused with the term residual oil, which means the oily residue left in the stills after distilling off any portion of the original charge. The residuums here referred to are the residues left in the stills 40 after distilling off or destroying the oily portion of the charge but without carrying the distillation to the point of producing coke. They are heavy, tacky, dark green or black substances, solid or semi-solid at room temperature and are used for road building and the like not for lubrication.

In the quenching of steel the art has generally used a mineral oil bath having low viscosity, i. e. a viscosity of not over 150 seconds at 100° F. on a Saybolt viscosimeter,

and a flash point of from 300° to 450° measured by the Cleveland cup method. Low-viscosity oil is preferred for quenching because the lower the viscosity the less of it adheres to the steel parts upon removal from the bath, consequently there is less waste from drippage, and also oils of low viscosity are generally believed to give more rapid cooling of the steel than those of high viscosity. But since the cooling bath is unavoidably heated to a high temperature by the hot steel immersed in it, oils for such uses must have a sufficiently high flash point to avoid ignition, and a workable flash point has largely determined the viscosity characteristic; viscosity normally rising with flash point.

In quenching steel for most purposes it is desirable to cool it rapidly through its critical temperature, and thereafter at a slower rate. Water quenches quite rapidly and is desirable in that respect, but it has the disadvantage that the cooling rate is too rapid at lower steel temperatures. Oil, however, has a markedly decelerating rate of cooling, 70 and for steel below 700° F. The cooling curve tends to flatten out. That is, the rate of cooling is materially slower than at higher temperatures. Oil quenching improves the physical characteristics of the steel for most 75 uses, and it is because of this advantage that oil is used in spite of its relatively greater expense as compared to water. But in the initial stage of quenching the relatively slow cooling effect of the oil bath is not an advantage. Mineral oil baths have been improved to a slight extent by increasing their initial quenching rate by addition of animal oils, but these are relatively expensive, and therefore materially increase the cost of 80 quenching oil so treated or blended.

The present invention provides a simple and inexpensive way of increasing the initial quenching speeds of low-viscosity oil, without changing the desirable characteristics 85 just above referred to.

I have discovered that the residuums obtained from the distillation of mineral oils are much more effective for increasing the initial quenching speed of low-viscosity low- 100

flash mineral oils than are much greater quantities of high-viscosity high-flash mineral oils themselves. I have found that apparently the element which increases the initial quenching speed of oils does not pass over by distillation, but remains in the residuum of such a process. The residuum from the vacuum process of distilling oils are black or dark green products, tacky, usually solid at room temperature, and they are completely and permanently soluble in low viscosity mineral oils. In addition they are very cheap, being in effect a waste product of oil distillation. A comparatively small quantity of such residuum added to quenching oil of low viscosity low flash point will greatly increase its initial quenching rate, without increasing the cost of the compound as compared to the base oil to which the residuum is added.

I have found that the addition of 5% of the solid residuum of vacuum distillation of mineral oils to the usual low-viscosity low-flash mineral quenching oils as a base, raises the viscosity of the mixture only slightly, but produces an oil having a higher initial quenching rate for red hot steel than can be produced by adding twice as much high-viscosity high-flash oil as described in Patent 1,535,879, and much more than by adding the usual quantities of animal or vegetable oils. Moreover the said residuum is completely and permanently soluble in the low-viscosity quenching oil, whereas the steam refined cylinder stock referred to in the patent shows a tendency to settle out upon long standing. The residuum product is cheaper, and since comparatively a half or less in quantity may be used, the expense of treating the base quenching oil by the present process is cheaper than that described in the said patent.

It appears probable, from my experiments and discoveries, that the substance which is effective in increasing the initial quenching rate of low-viscosity mineral oils is not merely a mineral oil of high viscosity and high flash point, but rather some substance which is in the accumulated residuum left by the petroleum distillation process. Consequently the more concentrated by distillation the residuum is, the more quantitatively effective it appears to be for raising the initial quenching rate of the base oil to which it is to be added. Apparently the effective constituent does not pass over with the distillate.

While the residuum products of atmospheric distillation of oil have a considerable effectiveness as additional agents to quenching oils for the purpose of increasing the initial quenching rate, they are not so effective as the residuum of the vacuum process, and they are objectionable on account of the substantial amount of tar which is included in such residuum. Tar sinks to the bottom of

a quenching bath and may cause trouble in commercial operation.

The discoveries set forth in the prior patent above mentioned have proved practical and valuable in commercial use, and the present discovery is an improvement and extension thereof, involving a material cheapening of the process, and a material improvement of the product, due to the increased initial quenching rate and more complete solubility of the residuum product, and stability of the union thereof with the low-viscosity quenching oil.

I claim:

1. A quenching oil comprising a low-viscosity mineral oil combined with a lesser amount of the non-liquid residuum resulting from distillation of a mineral oil. 80
2. A quenching oil comprising a low-viscosity mineral oil combined with a lesser amount of the residuum resulting from distillation of a mineral oil in vacuo. 85
3. A quenching oil comprising a base of low-viscosity low-flash mineral oil with a smaller amount of the non-liquid residuum resulting from distilling mineral oil in vacuo dissolved in said base. 90
4. The method of increasing the initial quenching speed of a low-flash low-viscosity mineral oil, consisting in combining therewith a smaller amount of the residuum product resulting from distillation of a mineral oil. 95
5. The method of increasing the initial quenching speed of a low-flash low-viscosity mineral oil, consisting in dissolving therein a smaller amount of the solid residuum resulting from distilling a mineral oil in vacuo. 100

In testimony whereof, I sign my name.

HUGH RODMAN.

105

110

115

120

125

130